

V. H. EMERSON, G. A. MANWARING & J. K. REYNARD.  
COMPOSITE DISK SOUND RECORD.  
APPLICATION FILED JUNE 29, 1905.

1,102,253.

Patented July 7, 1914.

Fig.1



Fig. 2



Fig. 3



Victor H. Emerson,  
George A. Manwaring, and  
James K. Reynard,  
Inventors.

Witnesses  
Raphael Ketter  
R. L. Scott

By their Attorneys:  
Mauro, Cameron, Lewis, & Marcell

# UNITED STATES PATENT OFFICE.

VICTOR H. EMERSON, OF NEW YORK, N. Y., GEORGE A. MANWARING, OF BAYONNE, NEW JERSEY, AND JAMES K. REYNARD, OF NEW YORK, N. Y., ASSIGNEES TO AMERICAN GRAPHOPHONE COMPANY, OF BRIDGEPORT, CONNECTICUT, A CORPORATION OF WEST VIRGINIA.

## COMPOSITE-DISK SOUND-RECORD.

1,102,253.

Specification of Letters Patent.

Patented July 7, 1914.

Application filed June 29, 1905. Serial No. 267,598.

*To all whom it may concern:*

Be it known that we, VICTOR H. EMERSON, GEORGE A. MANWARING, and JAMES K. REYNARD, citizens of the United States, and residents of New York city, New York; Bayonne, Hudson county, New Jersey, and New York city, New York, respectively, have invented a new and useful Improvement in Composite-Disk Sound-Records, which improvement is fully set forth in the following specification.

This invention relates to sound-records impressed in disks or tablets, and more particularly to the composite tablet and the manner of building up the same, and the method of making the record.

The invention will best be understood by describing in detail the successive steps employed in producing the article.

The drawings annexed hereto, as part of the specification, are sectional views exaggerated in thickness.

Figure 1 shows a pair of rollers through which is passing a matrix and the unfinished record-tablet; Fig. 2 represents a press operating upon the same; and Fig. 3 is the finished article.

The body of our tablet is built up of alternating layers of very thin paper and a "glue," constituting what is known in the stereotypers art as a "flong." This "glue" contains copal, starch, gluten, gum tragacanth, and alum (to prevent fermentation and to harden), and is not in itself new with us. We proceed by placing a sheet of very thin paper upon a flat surface, then apply a liberal coating of this glue, then spread over this a second sheet of paper followed by a second layer of the glue, and so on. Upon the last layer of the glue we place, instead of the ordinary thin sheet of paper, a specially prepared sheet. This latter is a thin sheet of paper coated with a suitable "paint" which is susceptible of receiving and retaining the impressions contained in the sound-record matrix, and this material must also be waterproof or water-insoluble. Preferably this "paint" consists of a solution containing celluloid and shellac with rotten stone. This solution in itself forms no part of the present invention. This solution or its equivalent is applied in one or more coats to the sheet of paper and allowed

to become dry and seasoned. The facing-paper already thus prepared is placed upon top of the "flong" above referred to, to constitute the facing of our new record-tablet.

In the drawings, A represents the "flong," made up of a plurality of very thin sheets of paper having intermediate layers of the "blue"; and B represents the facing-sheet containing upon its outer surface a coat of the "paint" above referred to. This composite tablet A B is then placed upon a suitable record-matrix C, with the facing B adjacent to the matrix-surface; a felt cloth D, about one inch thick, is laid upon the back (top) of the flong; and the whole is passed under heated rollers E. The action of the rollers serves to impress into the facing B the irregularities of the matrix-surface, and likewise forces out much of the water from the "flong." As the next step, we place the matrix and partly compressed and dried flong, as a whole, in a suitably heated press F. Thereafter, it is removed from the press and the finished record A' B is separated from the matrix. This finished article contains in the surface B a correct and permanent copy of the original sound-record from which the matrix has been obtained, and is durable and nonwarpable. It will be observed that water is the medium in which the glue is dissolved, and that neither as water nor when changed into steam will it affect the "paint" upon the facing B. During the rolling and pressing, under the heat of the rollers and press, the water is forced out in the form of steam and is partly absorbed by the felt, so as to leave the tablet A' B perfectly dry and hard. The completed article A' B will then be finished by waterproofing its back and edge. This system constitutes a radical departure in the production of sound-records: heretofore impressed sound-records have been made by treating a material which becomes soft and plastic under heat and pressure, whereas, our present system deals with a soft and plastic material which becomes hard and set under heat and pressure.

We do not limit ourselves to the precise ingredients or methods employed, having given detailed descriptions merely for the sake of clearness.

Having thus described our invention, we claim:

1. As an article of manufacture a sound-record consisting of a composite tablet composed of a plurality of sheets of very thin paper, the outer sheet having a facing of suitable "paint" containing celluloid and shellac in which the record proper, is impressed and all of said sheets united and impregnated with a suitable "glue."
2. As an article of manufacture, a sound-record consisting of a composite tablet composed of a plurality of sheets of very thin paper, the outer sheet having a facing of

superior sound-record material in which the record proper is impressed and all of said sheets being united and impregnated with a suitable glue.

In testimony whereof we have signed this specification in the presence of two subscribing witnesses.

VICTOR H. EMERSON.  
GEORGE A. MANWARING.  
JAMES K. REYNARD.

Witnesses:

C. A. L. MASSIE,  
W. H. HARTING.